# EUROPEAN PATENT SPECIFICATION

(11) **EP 0 592 118 B1**
(45) Date of publication and mention of the grant of the patent: **31.07.1996**
(21) Application number: 93307345.4
(22) Date of filing: 17.09.1993
(51) Int. Cl.: C23F 11/14

(54) **Method of controlling corrosion and biological matter in copper and copper alloy cooling water systems**
Verfahren zur Korrosions- und biologischen Substanzkontrolle in Kühlwassersystemen aus Kupfer und Kupferlegierungen
Méthode pour contrôler la corrosion et les matières biologiques dans des systèmes d'eau en cuivre et en alliage de cuivre

(30) Priority: 08.10.1992 US 958553
(43) Date of publication of application: 13.04.1994
(73) Proprietor: NALCO CHEMICAL COMPANY, Naperville Illinois 60563-1198 (US)
(72) Inventor: Lu, Frank F Y, Naperville, Illinois 60564 (US)
(74) Representative: Harrison, David Christopher

(56) References cited:
- EP-A- 0 462 809
- EP-A- 0 478 247
- EP-A- 0 479 572
- GB-A- 933 979

## Description

This invention relates generally to corrosion control and, more particularly, to a method of controlling corrosion of copper and copper alloys in cooling water systems, in the presence of oxidizing biocides.

Corrosion occurs when metals are oxidized to their respective soluble ions or insoluble salts. Metal loss due to solubilization can cause the structural integrity of the system to deteriorate over time. This can cause leakage between the water system and process streams. Also, the formation of insoluble salts in the corrosion process can produce a build-up of deposits which impede heat transfer and fluid flow.

Triazoles, such as tolyltriazole and benzotriazole are commonly used in cooling water systems as corrosion inhibitors for yellow metals, namely copper and copper alloys. Typically, triazoles are continuously fed into a recirculating cooling water system for inhibiting corrosion of copper and copper alloys. The purpose of this continuous feed is to maintain a low level of triazole first to form and then to maintain a protective triazole layer.

The continuous feed method, however, is too expensive to apply to once-through and high blowdown rate cooling water systems since large amounts of water are discharged from these systems in a short period of time. It would be both economically and environmentally unsound to continuously discharge such high volumes of triazole-loaded cooling water.

US-A-4,744,950 discloses the use of an alkyl benzotriazole to form a protective film on copper and copper alloys in cooling water systems by intermittently feeding the alkyl benzotriazole into once-through and high blowdown rate cooling water systems. While it is claimed in this patent that a corrosion inhibitive film is formed which will stand up to overfeeds of oxidizing biocides, it is also acknowledged that corrosion inhibitive films formed using benzotriazole and tolytriazole will be destroyed in the presence of the oxidizing biocides.

Oxidizing biocides are commonly added to cooling water systems. They are an inexpensive, yet effective means by which to control the formation of biological matter such as algae and bacteria. Chlorinating and brominating agents, which are the most widely used biocides in the cooling water treatment industry, are commonly fed intermittently. Unfortunately, as already noted, oxidizing biocides disrupt tolyltriazole and benzotriazole corrosion inhibitive films. More particularly, chlorine (OClO⁻_{,}HClO) and bromine (OBrO⁻, HOBr) penetrate and attack prefilmed triazole surfaces, thereby destroying the effectiveness of such cuprous metal corrosion inhibitors. Tolyltriazole and benzotriazole protective films are especially susceptible to attack by oxidizing biocides.

Therefore, it would be highly desirable to develop a new method of controlling corrosion of copper and copper alloys in cooling water systems which is economically and environmentally acceptable and effective in the presence of oxidizing biocides.

EP-A-462809 and 478247 have attempted to solve this problem by providing complex alkoxybenzotriazole compositions which are stated to have improved tolerance to oxidizing biocides.

The present invention, on the other hand, involves a method of controlling corrosion and biological matter, especially in once-through and high blowdown rate cooling water systems, which establishes a protective triazole film on copper and copper alloy surfaces and is characterized by then intermittently introducing a combination of a low level of triazole and an oxidizing biocide. Additionally, the corrosion rates and copper concentrations in the system discharge should be continuously monitored to determine if the formation of subsequent protective triazole films on the copper or copper alloy is required, and sufficient triazole should then be added, as required.

The addition of the triazole concomitantly with the oxidizing biocide surprisingly and effectively overcomes the loss of triazole protection formerly encountered when oxidizing biocides were used alone. The present invention is thus economically appealing, environmentally acceptable, and effective in controlling not only corrosion, but biological matter, such as algae and bacteria, as well.

In the drawings:
Figure 1 is a plot of the corrosion rate of copper versus the treatment cycle, as discussed in Example 1;
Figure 2 is a plot of the corrosion rate of cooper versus the treatment cycle, as discussed in Example 2;
Figure 3 is a plot of the corrosion rate of admiralty versus the treatment cycle, as discussed in Example 3; and
Figure 4 is a plot of the corrosion rate of admiralty versus the treatment cycle, as discussed in Example 4.

In the practice of the present invention, a protective triazole film is established on a copper or copper alloy surface. Tolyltriazole, benzotriazole, or C₁ to C₁₂ alkyl substituted benzotriazoles may be used as the cuprous metal corrosion inhibitor. Tolyltriazole is preferred. The triazole should be present in the system water at a level ranging from about 0.5 to 50 ppm by weight for a time period of at least about 2 hours, and preferably in the range of about 3 to 5 ppm for about 4 to 48 hours.

After the protective triazole film has formed on the copper or copper alloy surface, further triazole application is not necessary until the need for intermittent triazole/oxidizing biocide arises. This will be determined on a case-by-case basis by, e.g., monitoring the bacterial count in the cooling system water to determine when to begin the feed and how often to repeat it. Oxidizing biocides from the group comprising chlorine (OCl0⁻ , HCl0), bromine (OBrO⁻ , HOBr), NaOCl and NaOBr may be used at this stage in the treatment. In a preferred embodiment, NaOCl or NaOBr is used.

In accordance with the intermittent oxidizing biocide treatment step, a low level of triazole is introduced into the cooling water system along with the oxidizing biocide. Tolyltriazole, benzotriazole, C₁ to C₁₂ alkyl substituted benzotriazoles, or other commercially available triazoles may be used as the cuprous metal corrosion inhibitor. Tolyltriazole is preferred. A low level of triazole, as prescribed below in Table 1, is added at the same time as the oxidizing biocide:

**Table 1**

| Tolyltriazole Dosage During Oxidizing Biocide Treatments (ppm) | | | |
|---|---|---|---|
| Metallurgy | Broad Range | Preferred Range | Most Preferred Range |
| Copper | 0.1-50 | 0.2-5 | 0.2 - 2.0 |
| Admiralty (FRC* = 1 ppm) | 0.1-50 | 0.2-5 | 0.5 - 2.0 |
| Admiralty (FRC* = 10 ppm) | 0.1-50 | 0.2-5 | 1.0 - 2.0 |
| Al - bronze | 0.1-50 | 0.2-5 | 1.0 - 2.0 |
| Cu-Ni 90/10 | 0.1-50 | 0.2-5 | 1.0 - 2.0 |

| | | | |
|---|---|---|---|
| *FRC - Free Residual Chlorine | | | |

The corrosion rates and copper concentrations in the discharge are then continuously monitored with a suitable device such as a corrater, until it is determined that the formation of another subsequent protective triazole film on the copper or copper alloy is required. When this occurs, sufficient triazole is added to raise the level to at least about 0.5 to 50 ppm for at least about 2 hours, and preferably to the range of about 3 to 5 ppm for about 4 to 48 hours.

### EXAMPLES

The following examples are intended to be illustrative of the present invention and to teach one of ordinary skill how to make and use the invention. These examples are not intended to limit the invention or its protection in any way.

The examples explained below are bench-top experimental tests which simulate intermittent feed programs, with and without the simultaneous addition of tolyltriazole.

### EXAMPLE 1

Copper electrodes were prefilmed by immersing them in a 5 ppm tolyltriazole solution for about 20 hours. The prefilmed electrodes were then subjected to 12 cycles of intermittent NaOBr treatment. Each cycle included a 2 hour immersion in a 1 ppm free residual chlorine (FRC) NaOBr solution followed by a 22 hour immersion in tap water, which was aerated at room temperature.

Corrosion rates were then obtained by taking linear polarization resistance measurements in the tap water. The polarization resistance data were converted to mpy (mils per year of metal loss) using equation (1), where Rp represents polarization resistance.$\text{mpy =} \frac{\text{10.58}}{{\text{Rp (Kohm x cm}}^{\text{2}} \text{)}}$ In terms of mm per year the expression would have a numerator of 0.27 instead of 10.58.

The corrosion rate at each of the 12 cycles of intermittent NaOBr treatment is plotted in FIGURE 1. The corrosion rates were unacceptable, as will be evident to those skilled in the art.

### EXAMPLE 2

The same procedure as described in Example 1 was followed, except that each cycle also included the simultaneous addition of 0.5 ppm tolyltriazole with the 1 ppm (FRC) NaOBr solution.

FIGURE 2 illustrates that the corrosion rates decreased significantly when the tolyltriazole was added simultaneously with the NaOBr. A comparison of FIGURES 1 and 2 indicates that superior corrosion control is achieved when a low level of tolyltriazole is simultaneously added during intermittent NaOBr treatment.

### EXAMPLE 3

Admiralty electrodes were prefilmed by immersing them in a 5 ppm tolytriazole or 5 ppm butylbenzotriazole solution for about 20 hours. The blank was a freshly polished admiralty electrode with 600 grit SiC which was etched with 10% H₂SO₄.

The prefilmed and blank electrodes were then subjected to 6 cycles of intermittent NaOBr treatment. Each cycle included a 2 hour immersion in a 10 ppm (FRC) NaOBr solution followed by a 22 hour immersion in tap water, which was aerated at room temperature.

The corrosion rates were determined as explained above in Example 1.

The corrosion rate at each of the 6 cycles of intermittent NaOBr treatment is plotted in FIGURE 3. The unacceptable corrosion rates will be evident to those skilled in the art.

### EXAMPLE 4

The same procedure as described in Example 3 was followed, except that each cycle also included the simultaneous addition of either 0.2 ppm tolyltriazole, 0.5 ppm tolytriazole, 1.0 ppm tolytriazole, or 2.0 ppm tolytriazole with the 10 ppm (FRC) NaOBr solution.

FIGURE 4 shows that the corrosion rates decreased significantly when the tolyltriazole was added simultaneously with the NaOBr. A comparison of FIGURES 3 and 4 indicates that superior corrosion control is achieved when a low level of tolyltriazole is introduced along with the intermittent NaOBr treatment.

While the present invention is described above in connection with preferred or illustrative embodiments, these embodiments are not intended to be exhaustive or limiting of the invention.

## Claims

1. A method of controlling corrosion of copper and copper alloys in cooling water systems comprising the steps of:
establishing a protective triazole film on the copper and copper alloy surfaces in the system; and then
intermittently introducing an oxidizing biocide into the cooling water system characterized in that a low level of triazole is introduced at the same time as the biocide.

2. The method of claim 1 including the steps of:
continuously monitoring corrosion rates and copper concentrations to determine the state of the protective triazole film on the copper or copper alloy; and
reestablishing the protective triazole film, when determined necessary, before introduction of the biocide and triazole.

3. The method of claim 1 in which the triazole is chosen from the group consisting of tolyltriazole, benzotriazole, and C₁ to C₁₂ alkyl substituted benzotriazoles.

4. The method of claim 3 in which the triazole is tolyltriazole.

5. The method of claim 1 in which the protective triazole film is formed by applying triazole at a level of 0.5 to 50 ppm by weight for a time period of at least about 2 hours.

6. The method of claim 5 in which the protective triazole film is formed by applying triazole at a level of 3 to 5 ppm by weight for a time period of 4-48 hours.

7. The method of claim 1 in which the level of triazole maintained by the introduction is from 0.2 to 5.0 ppm by weight.

8. The method of claim 7 in which the level of triazole is 0.2 to 2 ppm by weight.

9. The method of claim 1 in which the oxidizing biocide is chlorine (OClO⁻, HClO), bromine (OBrO⁻, HOBr), NaOCl, or NaOBr.

## Patentansprüche

1. Verfahren zur Hemmung der Korrosion von Kupfer und von Kupferlegierungen in Kühlwassersystemen, umfassend die folgenden Schritte:
Bilden eines schützenden Triazolfilms auf den Kupfer- und Kupferlegierungsoberflächen im System; und anschließende intermittierende Zufuhr eines oxidierenden Biozids in das Kühlwassersystem,
dadurch gekennzeichnet, daß eine geringe Menge an Triazol gleichzeitig mit dem Biozid eingebracht wird.

2. Verfahren nach Anspruch 1, umfassend die folgenden Schritte:
kontinuierliches Überwachen der Korrosionsraten und Kupferkonzentrationen, um den Zustand des schützenden Triazolfilms auf dem Kupfer oder der Kupferlegierung zu bestimmen; und
erneutes Bilden des schützenden Triazolfilms vor der Zufuhr von Biozid und Triazol, wenn sich dies als notwendig erweist.

3. Verfahren nach Anspruch 1, worin das Triazol aus der Gruppe bestehend aus Tolyltriazol, Benzotriazol und C₁-C₁₂-alkylsubstituierten Benzotriazolen ausgewählt wird.

4. Verfahren nach Anspruch 3, worin das Triazol Tolyltriazol ist.

5. Verfahren nach Anspruch 1, worin der schützende Triazolfilm durch den Einsatz von Triazol in einer Menge von 0,5-50 Gew.-ppm über einen Zeitraum von zumindest etwa 2 Stunden gebildet wird.

6. Verfahren nach Anspruch 5, worin der schützende Triazolfilm durch den Einsatz von Triazol in einer Menge von 3-5 Gew.-ppm über einen Zeitraum von 448 Stunden gebildet wird.

7. Verfahren nach Anspruch 1, worin die durch die Zufuhr aufrechterhaltene Menge an Triazol 0,2-5,0 Gew.-ppm beträgt.

8. Verfahren nach Anspruch 7, worin die Menge an Triazol 0,2-2 Gew.-ppm beträgt.

9. Verfahren nach Anspruch 1, worin das oxidierende Biozid Chlor (OClO⁻, HClO), Brom (OBrO⁻, HOBr), NaOCl oder NaOBr ist.

## Revendications

1. Méthode de contrôle de la corrosion d'alliages de cuivre et de cuivre dans des systèmes de refroidissement d'eau comprenant les étapes de :
établissement d'un film protecteur de triazole sur les surfaces de cuivre et d'alliages de cuivre dans le système; et ensuite
introduction par intermittence d'un biocide oxydant dans le système de refroidissement d'eau caractérisée en ce qu'un faible niveau de triazole est introduit en même temps que le biocide.

2. Méthode selon la revendication 1 incluant les étapes de :
contrôle en continu des taux de corrosion et des concentrations en cuivre pour déterminer l'état du film de triazole protecteur sur le cuivre ou l'alliage de cuivre; et
rétablissement du film de triazole protecteur, lorsque déterminé nécessaire, avant introduction du biocide et du triazole.

3. Méthode selon la revendication 1 dans laquelle le triazole est choisi dans le groupe consistant du tolyltriazole, du benzotriazole, et des benzotriazoles substitués par un alkyle en C₁ à C₁₂.

4. Méthode selon la revendication 3 dans laquelle le triazole est le tolyltriazole.

5. Méthode selon la revendication 1 dans laquelle le film de triazole protecteur est formé par application de triazole à un niveau de 0,5 à 50 ppm en poids pendant une période de temps d'au moins environ 2 heures.

6. Méthode selon la revendication 5 dans laquelle le film de triazole protecteur est formé par application de triazole à un niveau de 3 à 5 ppm en poids pendant une période de temps de 4 à 48 heures.

7. Méthode selon la revendication 1 dans laquelle le niveau de triazole maintenu par l'introduction est de 0,2 à 5,0 ppm en poids.

8. Méthode selon la revendication 7 dans laquelle le niveau de triazole est de 0,2 à 2 ppm en poids.

9. Méthode selon la revendication 1 dans laquelle le biocide oxydant est le chlore (OClO⁻, HClO), le brome (OBrO⁻, HOBr), NaOCl, ou NaOBr.
